

## United States Patent [19]

Buckley et al.

[11] Patent Number: 4,479,999

[45] Date of Patent: Oct. 30, 1984

[54] FABRIC COMPRISING OF FUSIBLE AND INFUSIBLE FIBERS, THE FORMER COMPRISING A POLYMER WHICH IS CAPABLE OF FORMING AN ANISOTROPIC MELT PHASE

[75] Inventors: Alan Buckley, Berkeley Heights; Paul E. McMahon, Chatham, both of N.J.

[73] Assignee: Celanese Corporation, New York, N.Y.

[21] Appl. No.: 368,491

[22] Filed: Apr. 15, 1982

[51] Int. Cl. 3 B32B 27/12; B32B 27/36

[52] U.S. Cl. 428/245; 428/229; 428/271; 428/272; 428/273; 428/288; 428/294; 428/296; 428/408; 428/481; 428/902

[58] Field of Search 528/190; 428/288, 229, 428/272, 271, 273, 294, 296, 245, 481, 902, 408

[56] References Cited

U.S. PATENT DOCUMENTS

3,620,892 11/1971 Winklhofer et al. 428/197

|           |         |                    |         |
|-----------|---------|--------------------|---------|
| 3,975,487 | 8/1976  | Cottes et al. .... | 264/236 |
| 4,183,895 | 1/1980  | Luise ....         | 528/191 |
| 4,362,777 | 12/1982 | Miller ....        | 428/288 |
| 4,368,234 | 1/1983  | Palmer et al. .... | 428/245 |

FOREIGN PATENT DOCUMENTS

1228573 4/1971 United Kingdom .

Primary Examiner—James C. Cannon  
Attorney, Agent, or Firm—Burns, Doane, Swecker & Mathis

[57] ABSTRACT

An improved fabric is provided comprised of fusible and infusible fibers. The fusible fibers comprise thermotropic liquid crystal polymers (i.e., polymers which are capable of forming an anisotropic melt phase). When the liquid crystal fibers are heated, they fuse to adjacent infusible fibers without any substantial loss of the orientation which was imparted to the same during melt extrusion. A fabric of enhanced strength and stiffness is thus formed in comparison to a fabric which employs conventional thermoplastic polymers which do not form an anisotropic melt phase.

34 Claims, No Drawings

FABRIC COMPRISING OF FUSIBLE AND  
INFUSIBLE FIBERS, THE FORMER  
COMPRISING A POLYMER WHICH IS CAPABLE  
OF FORMING AN ANISOTROPIC MELT PHASE

CROSS-REFERENCE TO RELATED  
APPLICATIONS

This application is related to U.S. patent application Ser. No. 319,525, filed Nov. 9, 1981, of Alan Buckley and Gordon W. Calundann entitled "Non-Woven Articles Comprised of Thermotropic Liquid Crystal Polymer Fibers."

BACKGROUND OF THE INVENTION

The present invention relates to fabrics fabricated from infusible fibers and fusible fibers of thermotropic liquid crystal polymers.

Fabrics have been produced comprised of fusible and infusible fibers. The fusible fibers, typically comprised of thermoplastic polymeric materials, are initially woven together with the infusible fibers into a fabric, with the fabric subsequently being heat treated at a temperature above the melting point of the fusible fibers. The fusible fibers thus become thermally bonded to adjacent infusible fibers and, in effect, serve as a matrix therefore. See, for example, U.S. Pat. No. 3,620,892 and British Patent Nos. 1,228,573 and 1,260,409. Conventional thermoplastic materials possess certain disadvantages, however, in that the physical characteristics of the thermoplastic material (e.g., strength and polymer orientation within the fibers) are significantly lessened as a result of the thermal bonding of the fibers. It is therefore desirable to provide a fabric comprised of fusible and infusible materials wherein the fusible material retains its desirable physical characteristics subsequent to being heated above its melting temperature.

It is also known to those skilled in the art that the heat treatment of shaped articles of liquid crystal polymers increases the melting temperature, molecular weight and mechanical properties of the polymer. See, for example, U.S. Pat. Nos. 3,975,487; 4,183,895; and 4,247,514.

OBJECTS AND SUMMARY OF THE  
INVENTION

It is therefore an object of the present invention to provide a fabric containing fibers comprised of a thermoplastic polymer which polymer retains its desirable mechanical properties subsequent to heat treatment thereof at a temperature above the melting temperature of the polymer.

It is also an object of the present invention to provide a fabric containing both fusible and infusible fibers wherein the fusible fibers can be thermally bonded to the infusible fibers without loss of desirable mechanical properties.

It is also an object of the present invention to provide a fabric which exhibits desirable thermal stability and chemical and solvent resistance.

In accordance with the present invention there is thus provided a fabric which exhibits thermal stability and chemical and solvent resistance comprised of fusible and infusible fibers, said fusible fibers being thermally bonded to the infusible fibers and comprised of a poly-

mer which is capable of forming an anisotropic melt phase.

DETAILED DESCRIPTION OF THE  
INVENTION

It has been found that thermotropic liquid crystal polymers are uniquely suited for use as fusible fibers in fabrics comprised of fusible and infusible fibers. Thermotropic liquid crystal polymers retain their anisotropic characteristics in the melt phase such that the polymers remain highly oriented. Fabrics comprised of thermotropic liquid crystal fibers retain residual strength characteristics subsequent to being subjected to heat treatment to fuse the thermotropic fibers to adjacent fibers.

For purposes of the present invention, fusible fibers are those fibers which can be reduced to a liquid state or melted without significant degradation of the polymer or loss of its properties upon resolidification. The fusible fibers are also comprised of a polymer which is capable of forming an anisotropic melt phase at a temperature which is preferably below about 600° C. and most preferably below about 400° C. Infusible fibers are those fibers which either (1) cannot be reduced to a liquid state, (2) can be reduced to a liquid state only with significant thermal and/or oxidative degradation, or (3) can only be reduced to a liquid state at a temperature in excess of about 700° C. For example, carbon fibers will sublime and/or erode by oxidation upon being subjected to excessive temperatures and are thus deemed to be infusible by character. In addition, glass fibers are deemed to be infusible for purposes of the present invention since they generally melt at a temperature in excess of about 700° C. Similarly, lyotropic liquid crystal polymers are deemed to be infusible since they are solution-processable and not melt-processable. An exemplary lyotropic liquid crystal polymer is poly(p-phenylene terephthalamide) marketed by DuPont under the trademark Kevlar.

Thermotropic liquid crystal polymers are polymers which are liquid crystalline (i.e., anisotropic) in the melt phase. These polymers have been described by various terms, including "liquid crystalline", "liquid crystal" and "anisotropic". Briefly, the polymers of this class are thought to involve a parallel ordering of the molecular chains. The state wherein the molecules are so ordered is often referred to either as the liquid crystal state or the nematic phase of the liquid crystalline material. These polymers are prepared from monomers which are generally long, flat and fairly rigid along the long axis of the molecule and commonly have chain-extending linkages that are either coaxial or parallel.

Such polymers readily form liquid crystals (i.e., exhibit anisotropic properties) in the melt phase. Such properties may be confirmed by conventional polarized light techniques whereby crossed polarizers are utilized. More specifically, the anisotropic melt phase may be confirmed by the use of a Leitz polarizing microscope at a magnification of 40 $\times$  with the sample on a Leitz hot stage and under nitrogen atmosphere. The polymer is optically anisotropic; i.e., it transmits light when examined between crossed polarizers. Polarized light is transmitted when the sample is optically anisotropic even in the static state.

Thermotropic liquid crystal polymers include but are not limited to wholly and non-wholly aromatic polyesters, aromatic-aliphatic polyesters, aromatic poly-

zomethines, aromatic polyester-carbonates and aromatic and non-wholly aromatic polyester-amides.

The aromatic polyesters and poly(ester-amide)s are considered to be "wholly" aromatic in the sense that each moiety present in the polyester contributes at least one aromatic ring to the polymer backbone and which enable the polymer to exhibit anisotropic properties in the melt phase. Such moieties may be derived from aromatic diols, aromatic amines, aromatic diacids and aromatic hydroxy acids. Moieties which may be present in the thermotropic liquid crystal polymers employed in the present invention (wholly or non-wholly aromatic) include but are not limited to the following:



Preferably, the thermotropic liquid crystal polymers which are employed comprise not less than about 10 mole percent of recurring units which include a naphthalene moiety. Preferred naphthalene moieties include 6-oxy-2-naphthoyl, 2,6-dioxynaphthalene and 2,6-dicarboxynaphthalene.

Specific examples of suitable aromatic-aliphatic polyesters are copolymers of polyethylene terephthalate and hydroxybenzoic acid as disclosed in *Polyester X7G-A Self Reinforced Thermoplastic*, by W. J. Jackson, Jr., H. F. Kuhfuss, and T. F. Gray, Jr., 30th Anniversary Technical Conference, 1975 Reinforced Plastics/Composites Institute, The Society of the Plastics Industry, Inc., Section 17-D, Pages 1-4. A further disclosure of such copolymers can be found in "Liquid Crystal Polymers: I. Preparation and Properties of p-Hydroxybenzoic Acid Copolymers," *Journal of Polymer Science, Polymer Chemistry Edition*, Vol. 14, pp. 2043-58 (1976), by W. J. Jackson, Jr., and H. F. Kuhfuss. The above-cited references are herein incorporated by reference in their entirety.

Aromatic polyazomethines and processes of preparing the same are disclosed in the U.S. Pat. Nos. 3,493,522; 3,493,524; 3,503,739; 3,516,970; 3,516,971;

3,526,611; 4,048,148; and 4,122,070. Each of these patents is herein incorporated by reference in its entirety. Specific examples of such polymers include poly(nitrilo-2-methyl-1,4-phenylenenitriloethylidyne-1,4-phenyleneethylidyne); poly(nitrolo-2-methyl-1,4-phenylenenitrilomethylidyne-1,4-phenylene-methylidyne); and poly(nitrilo-2-chloro-1,4-phenylenenitrilomethylidyne-1,4-phenylenemethylidyne).

10 Aromatic polyester-carbonates are disclosed in U.S. Pat. No. 4,107,143 and 4,284,757, which are herein incorporated by reference in their entirety. Examples of such polymers include those consisting essentially of p-oxybenzoyl units, p-dioxyphenyl units, dioxy carbonyl units, and terephthoyl units.

15 Aromatic polyester-amides and processes of preparing the same are disclosed in the U.S. Pat. No. 4,182,842. Further disclosure of such copolymers can be found in "Liquid Crystal Polymers: III Preparation of Properties of Poly(Ester Amides) from p-Aminobenzoic Acid and Poly(Ethylene Terephthalate)," *Journal of Applied Polymer Science*, Vol. 25 pp. 1685-1694 (1980), by W. J. Jackson, Jr., and H. F. Kuhfuss. The above cited references are herein incorporated by reference in their entirety.

20 The liquid crystal polymers which are preferred for use in the present invention are the thermotropic wholly aromatic polyesters. Recent publications disclosing such polyesters include (a) Belgian Pat. Nos. 828,935 and 828,936, (b) Dutch Pat. No. 7505551, (c) West German Pat. Nos. 2,520,819, 2,520,820, and 2,722,120, (d) Japanese Pat. Nos. 43-223, 2132-116, 3017-692, and 3021-293, (e) U.S. Pat. Nos. 3,991,013; 3,991,014; 4,057,597; 4,066,620; 4,075,262; 4,118,372; 4,146,702; 4,153,779; 4,156,070; 4,159,365; 4,169,933; 4,181,792; 4,188,476; 4,226,970; 4,201,856; 4,232,143; 4,232,144; 4,245,082; and 4,238,600; and (f) U. K. Application No. 2,002,404.

25 Wholly aromatic polymers which are preferred for use in the present invention include wholly aromatic polyesters and poly(ester-amide)s which are disclosed in commonly-assigned U.S. Pat. Nos. 4,067,852; 4,083,829; 4,130,545; 4,161,470; 4,184,996; 4,219,461; 4,230,817; 4,238,598; 4,238,599; 4,244,433; 4,256,624; 4,279,803; 4,299,756; 4,330,457; 4,339,375; 4,341,688; 4,351,917; 4,351,918; and 4,355,132. The disclosures of all of the above-identified commonly-assigned U.S. patents and applications are herein incorporated by reference in their entirety. The wholly aromatic polyesters and poly(ester-amide)s disclosed therein typically are capable of forming an anisotropic melt phase at a temperature below approximately 400° C., and preferably below approximately 350° C.

30 The thermotropic liquid crystal polymers including wholly aromatic polyesters and poly(ester-amide)s which are suitable for use in the present invention may be formed by a variety of ester-forming techniques whereby organic monomer compounds possessing functional groups which, upon condensation, form the requisite recurring moieties are reacted. For instance, the functional groups of the organic monomer compounds may be carboxylic acid groups, hydroxyl groups, ester groups, acyloxy groups, acid halides, 35 amine groups, etc. The organic monomer compounds may be reacted in the absence of a heat exchange fluid via a melt acidolysis procedure. They, accordingly, may be heated initially to form a melt solution of the

reactants with the reaction continuing as said polymer particles are suspended therein. A vacuum may be applied to facilitate removal of volatiles formed during the final stage of the condensation (e.g., acetic acid or water).

Commonly-assigned U.S. Pat. No. 4,083,829, entitled "Melt Processable Thermotropic Wholly Aromatic Polyester," describes a slurry polymerization process which may be employed to form the wholly aromatic polyesters which are preferred for use in the present invention. According to such a process, the solid product is suspended in a heat exchange medium. The disclosure of this patent has previously been incorporated herein by reference in its entirety. Although that patent is directed to the preparation of wholly aromatic polyesters, the process may also be employed to form poly(ester-amide)s.

When employing either the melt acidolysis procedure or the slurry procedure of U.S. Pat. No. 4,083,829, the organic monomer reactants from which the wholly aromatic polyesters are derived may be initially provided in a modified form whereby the usual hydroxy groups of such monomers are esterified (i.e., they are provided as lower acyl esters). The lower acyl groups preferably have from about two to about four carbon atoms. Preferably, the acetate esters of organic monomer reactants are provided. When poly(ester-amide)s are to be formed, an amine group may be provided as a lower acyl amide.

Representative catalysts which optionally may be employed in either the melt acidolysis procedure or in the slurry procedure of U.S. Pat. No. 4,083,829 include dialkyl tin oxide (e.g., dibutyl tin oxide), diaryl tin oxide, titanium dioxide, antimony trioxide, alkoxy titanium silicates, titanium alkoxides, alkali and alkaline earth metal salts of carboxylic acids (e.g., zinc acetate), the gaseous acid catalysts such as Lewis acids (e.g.,  $\text{BF}_3$ ), hydrogen halides (e.g.,  $\text{HCl}$ ), etc. The quantity of catalyst utilized typically is about 0.001 to 1 percent by weight based upon the total monomer weight, and most commonly about 0.01 to 0.2 percent by weight.

The wholly aromatic polyesters and poly(ester-amide)s suitable for use in the present invention tend to be substantially insoluble in common polyester solvents and accordingly are not susceptible to solution processing. As discussed previously, they can be readily processed by common melt processing techniques. Most suitable wholly aromatic polymers are soluble in pentafluorophenol to a limited extent.

The wholly aromatic polyesters which are preferred for use in the present invention commonly exhibit a weight average molecular weight of about 2,000 to 200,000, and preferably about 10,000 to 50,000, and most preferably about 20,000 to 25,000. The wholly aromatic poly(ester-amide)s which are preferred for use in the present invention commonly exhibit a molecular weight of about 5,000 to 50,000, and preferably about 10,000 to 30,000; e.g., 15,000 to 17,000. Such molecular weight may be determined by gel permeation chromatography and other standard techniques not involving the solutioning of the polymer, e.g., by end group determination via infrared spectroscopy on compression molded films. Alternatively, light scattering techniques in a pentafluorophenol solution may be employed to determine the molecular weight.

The wholly aromatic polyesters and poly(ester-amide)s additionally commonly exhibit an inherent viscosity (i.e., I.V.) of at least approximately 2.0 dl./g.,

e.g., approximately 2.0 to 10.0 dl./g., when dissolved in a concentration of 0.1 percent by weight in pentafluorophenol at 60° C.

For the purposes of the present invention, the aromatic rings which are included in the polymer backbones of the polymer components may include substitution of at least some of the hydrogen atoms present upon an aromatic ring. Such substituents include alkyl groups of up to four carbon atoms; alkoxy groups having up to four carbon atoms; halogens; and additional aromatic rings, such as phenyl and substituted phenyl. Preferred halogens include fluorine, chlorine and bromine. Although bromine atoms tend to be released from organic compounds at high temperatures, bromine is more stable on aromatic rings than on aliphatic chains, and therefore is suitable for inclusion as a possible substituent on the aromatic rings.

Especially preferred wholly aromatic polyesters and poly(ester-amide)s are those which are disclosed in above-noted U.S. Pat. Nos. 4,161,470, 4,184,996, 4,219,461, 4,256,624, 4,238,599 and 4,330,457.

The wholly aromatic polyester which is disclosed in U.S. Pat. No. 4,161,470 is a melt processable wholly aromatic polyester capable of forming in anisotropic melt phase at a temperature below approximately 350° C. The polyester consists essentially of the recurring moieties I and II wherein:



and



The polyester comprises approximately 10 to 90 mole percent of moiety I, and approximately 10 to 90 mole percent of moiety II. In one embodiment, moiety II is present in a concentration of approximately 65 to 85 mole percent, and preferably in a concentration of approximately 70 to 80 mole percent, e.g., approximately 75 mole percent. In another embodiment, moiety II is present in a lesser proportion of approximately 15 to 35 mole percent, and preferably in a concentration of approximately 20 to 30 mole percent. In addition, at least some of the hydrogen atoms present upon the rings optionally may be replaced by substitution selected from the group consisting of an alkyl group of 1 to 4 carbon atoms, an alkoxy group of 1 to 4 carbon atoms, halogen, phenyl, substituted phenyl, and mixtures thereof.

The wholly aromatic polyester which is disclosed in U.S. Pat. No. 4,184,996 is a melt processable wholly aromatic polyester capable of forming an anisotropic melt phase at a temperature below approximately 325° C. The polyester consists essentially of the recurring moieties I, II and III wherein:



The polyester comprises approximately 30 to 70 mole percent of the moiety I. The polyester preferably comprises approximately 40 to 60 mole percent of moiety I, approximately 20 to 30 mole percent of moiety II, and approximately 20 to 30 mole percent of moiety III. In addition, at least some of the hydrogen atoms present upon the rings optionally may be replaced by substitution selected from the group consisting of an alkyl group of 1 to 4 carbon atoms, an alkoxy group of 1 to 4 carbon atoms, halogen, phenyl, substituted phenyl, and mixtures thereof.

The wholly aromatic polyester which is disclosed in U.S. Pat. No. 4,238,599 is a melt processable polyester capable of forming an anisotropic melt phase at a temperature no higher than approximately 320° C. consisting essentially of the recurring moieties I, II, III and IV wherein:



where R is methyl, chloro, bromo, or mixtures thereof, and is substituted for a hydrogen atom present upon the aromatic ring, and wherein said polyester comprises approximately 20 to 60 mole percent of moiety I, ap-

proximately 5 to 18 mole percent of moiety II, approximately 5 to 35 mole percent of moiety III, and approximately 20 to 40 mole percent of moiety IV. The polyester preferably comprises approximately 35 to 45 mole percent of moiety I, approximately 10 to 15 mole percent of moiety II, approximately 15 to 25 mole percent of moiety III, and approximately 25 to 35 mole percent of moiety IV, with the proviso that the total molar concentration of moieties II and III is substantially identical to that of moiety IV. In addition, at least some of the hydrogen atoms present upon the rings optionally may be replaced by substitution selected from the group consisting of an alkyl group of 1 to 4 carbon atoms, an alkoxy group of 1 to 4 carbon atoms, halogen, phenyl, substituted phenyl, and mixtures thereof. This wholly aromatic polyester commonly exhibits an inherent viscosity of at least 2.0 dl./g., e.g., 2.0 to 10.0 dl./g., when dissolved in a concentration of 0.1 weight/volume percent in pentafluorophenol at 60° C.

The polyester disclosed in U.S. Pat. No. 4,219,461 is a melt processable wholly aromatic polyester which is capable of forming an anisotropic melt phase at a temperature below approximately 320° C. The polyester consists essentially of the recurring moieties I, II, III, and IV wherein:



wherein the polyester comprises approximately 20 to 40 mole percent of moiety I, in excess of 10 up to about 50 mole percent of moiety II, in excess of 5 up to about 30 mole percent of moiety III, and in excess of 5 up to about 30 mole percent of moiety IV. The polyester preferably comprises approximately 20 to 30 (e.g., approximately 25) mole percent of moiety I, approximately 25 to 40 (e.g., approximately 35) mole percent of moiety II, and approximately 15 to 25 (e.g., approximately 20) mole percent of moiety III and approximately 15 to 25 (e.g., approximately 20) mole percent of moiety IV. In addition, at least some of the hydrogen atoms present upon the rings optionally may be replaced by substitution selected from the group consisting of an alkyl group of 1 to 4 carbon atoms, an alkoxy group of 1 to 4 carbon atoms, halogen, phenyl, substituted phenyl, and mixtures thereof.

Moieties III and IV are preferably symmetrical in the sense that the divalent bonds which join these moieties to other moieties in the main polymer chain are sym-

metrically disposed on one or more aromatic rings (e.g., are para to each other or diagonally disposed when present on a naphthalene ring). However, non-symmetrical moieties, such as those derived from resorcinol and isophthalic acid, may also be used.

Preferred moieties III and IV are set forth in above-noted U.S. Pat. No. 4,219,461. The preferred dioxy aryl moiety III is:



and the preferred dicarboxy aryl moiety IV is:



The polyester disclosed in U.S. Pat. No. 4,256,624 is a melt processable wholly aromatic polyester which is capable of forming an anisotropic melt phase at a temperature below approximately 400° C. The polyester consists essentially of the recurring moieties I, II, and III wherein:



II is a dioxy aryl moiety of the formula  $-\text{O}-\text{Ar}-\text{O}-$  where Ar is a divalent radical comprising at least one aromatic ring, and



where Ar' is a divalent radical comprising at least one aromatic ring, and

wherein the polyester comprises approximately 10 to 90 mole percent of moiety I, approximately 5 to 45 mole percent of moiety II, and approximately 5 to 45 mole percent of moiety III. The polyester preferably comprises approximately 20 to 80 mole percent of moiety I, approximately 10 to 40 mole percent of moiety II, and approximately 10 to 40 mole percent of moiety III. The polyester more preferably comprises approximately 60 to 80 mole percent of moiety I, approximately 10 to 20 mole percent of moiety II, and approximately 10 to 20 mole percent of moiety III. In addition, at least some of the hydrogen atoms present upon the rings optionally may be replaced by substitution selected from the group consisting of an alkyl group of 1 to 4 carbon atoms, an alkoxy group of 1 to 4 carbon atoms, halogen, phenyl, substituted phenyl, and mixtures thereof.

As with moieties III and IV of the polyester disclosed in U.S. Pat. No. 4,219,461, moieties II and III of the 65 polyester described immediately above may be symmetrical or nonsymmetrical, but are preferably symmetrical.

Preferred moieties II and III are set forth in above-noted U.S. Pat. No. 4,256,624. The preferred dioxy aryl moiety II is:



and the preferred dicarboxy aryl moiety III is:



20 U.S. Pat. No. 4,330,457 discloses a melt processable poly(ester-amide) which is capable of forming an anisotropic melt phase at a temperature below approximately 400° C. The poly(ester-amide) consists essentially of the recurring moieties I, II, III and optionally IV wherein:



35 II is  $-\text{C}(=\text{O})-\text{A}-\text{C}(=\text{O})-$ , where A is a divalent radical comprising

at least one aromatic ring or a divalent transcyclohexane radical,

40 III is  $-\text{Y}-\text{Ar}-\text{Z}-$ , where Ar is a divalent radical comprising at least one aromatic ring, Y is O, NH,

or NR, and Z is NH or NR, where R is an alkyl group

of 1 to 6 carbon atoms or an aryl group; and

IV is  $-\text{O}-\text{Ar}'-\text{O}-$ , where Ar' is a divalent radical comprising

at least one aromatic ring;

45 and wherein said poly(ester-amide) comprises approximately 10 to 90 mole percent of moiety I, approximately 5 to 45 mole percent of moiety II, approximately 5 to 45 mole percent of moiety III, and approximately 0 to 40 mole percent of moiety IV. In addition, at least some of the hydrogen atoms present upon the rings optionally may be replaced by substitution selected from the group consisting of an alkyl group of 1 to 4 carbon atoms, an alkoxy group of 1 to 4 carbon atoms, halogen, phenyl, substituted phenyl, and mixtures thereof.

Preferred moieties II, III and IV are set forth in above-noted U.S. Pat. No. 4,330,457. The preferred dicarboxy aryl moiety II is:



the preferred moiety III is:



or



and the preferred dioxy aryl moiety IV is:



The fabric of the present invention is comprised of fibers of thermotropic liquid crystal polymers and infusible fibers. Infusible fibers suitable for use in the present invention include carbon fibers, glass fibers, asbestos fibers, boron fibers, alumina fibers, silicon carbide, borosilicatealumina fibers and lyotropic liquid crystal polymer fibers. Those infusible fibers which are preferred are carbon fibers and glass fibers. This listing is not intended to be all-inclusive since one skilled in the art can readily determine which infusible fibers may be advantageously used in the fabric of the present invention.

The fabric of the present invention may be formed by any suitable method and may be woven, knitted or non-woven. Preferably, the thermotropic liquid crystal polymer fibers are utilized in a woven fabric. For example, the infusible fibers may be utilized as the warp in the woven fabric and the fusible fibers may be utilized as the weft, or vice versa. It is also possible to mix fusible and infusible fibers in either or both of the warp and weft.

The fabric need not be woven per se but can also be constructed by layering the infusible and fusible fibers upon one another. Preferably, the respective types of fibers are placed in alternating layers such that a layer of fusible fibers is adjacent a layer of infusible fibers. See, for example, British Patent Nos. 1,228,573 and 1,260,409, herein both fully and completely incorporated by reference, wherein such an embodiment is disclosed, albeit not with fibers of liquid crystal polymers.

The fabric can also be provided by spray spinning a random web of fibers of a thermotropic liquid crystal polymer onto a layer of infusible fibers (e.g., a woven web of carbon fibers). In the alternative, melt spun fibers of a thermotropic liquid crystal polymer cut to appropriately short lengths can be slurried with a liquid which is a non-solvent for the polymer (e.g., water) and subsequently filtered onto a web of infusible fibers. It is also possible to provide a slurry of both fusible and infusible fibers which are then filtered onto a web or screen to form a random array of both fusible and infusible fibers.

The fibers can also be braided together or a sheet can be formed by filament winding by use of fusible and infusible fibers.

Upon being fabricated by appropriate means, the fabric is subjected to heat treatment to thermally bond

the fusible thermotropic liquid crystal polymer fibers to adjacent and/or intersecting fibers. The extent of the bonding can vary depending upon the end use contemplated and the physical form desired for the fabric. That is, the fabric need only be heat treated sufficiently to bond the fusible fibers to the extent desired. The fabric may also be heat treated to a greater extent such that the thermotropic liquid crystal polymer fibers serve as a more coherent matrix-like structure for the infusible fibers. Such thermal bonding preferably occurs with the application of pressure in order to ensure that sufficient bonding of the fibers occurs.

The fabric of the present invention can be comprised of various proportions of the fusible and infusible fibers.

For example, the fabric is preferably comprised of from about 5 to about 80 weight percent of infusible fibers and from about 20 to about 95 weight percent of thermotropic liquid crystal polymer fibers, and more preferably from about 40 to about 70 weight percent of infusible fibers and from about 30 to about 60 weight percent of thermotropic liquid polymer fibers.

The fabric possesses many advantageous characteristics due to the presence of thermotropic liquid crystal polymers therein. That is, since liquid crystal polymers are highly oriented as spun, the fibers which comprise the fabrics of the present invention possess relatively high tensile strength and modulus. Accordingly, fabrics comprised of such fibers similarly exhibit relatively high tenacity and modulus.

In addition, the fibers retain such tensile strength and modulus even upon being subjected to temperatures sufficient to melt the fibers due to the ability of the polymers to form an anisotropic melt phase. This is in direct contrast to conventional thermoplastic polymers which are not capable of forming an anisotropic melt and which lose their orientation upon being subjected to temperatures in excess of their melting temperature.

Typical thicknesses of the fabric range from 0.005 inch to 0.10 inch. In addition, reinforcement of the fabric in several directions is also possible by varying the direction of orientation of the fusible fibers (e.g., the fibers may be oriented at 0,  $\pm 45$  and  $90^\circ$  to one axis of the fabric).

The fabrics also benefit from other physical characteristics of thermotropic liquid crystal polymers such as resistance to chemical corrosion or solvation and high temperature stability due to the high melting temperatures of the fibers. Such fabrics thus are well suited for use in high temperature and/or otherwise destructive environments which would tend to degrade conventional fabrics.

The fabrics of the present invention can be employed as metal replacements where density and dynamic mechanical vibrations are factors. For instance, lighter weight aircraft/aerospace components can be made from the fabric. Moving parts for industrial equipment are also a suitable end use where the rate of motion is determined by fundamental part vibration characteristics.

The mechanical properties of the fabric produced in accordance with the present invention can be improved still further by subjecting the fabric to a heat treatment following formation thereof. The heat treatment improves the properties of the fabric by increasing the molecular weight of the liquid crystalline polymer which comprises certain of the fibers present within the fabric and increasing the degree of crystallinity thereof.

while also increasing the melting temperature of the polymer. Such heat treatment can also serve to bond the fibers together.

The fabric may be thermally treated in an inert atmosphere (e.g., nitrogen, carbon dioxide, argon, helium) or alternatively, in a flowing oxygen-containing atmosphere (e.g., air). The use of a non-oxidizing substantially moisture-free atmosphere is preferred to avoid the possibility of thermal degradation. For instance, the fabric may be brought to a temperature approximately 10 to 30 centigrade degrees below the melting temperature of the liquid crystal polymer, at which temperature the fibers remain a solid object. It is preferable for the temperature of the heat treatment to be as high as possible without equaling or exceeding the melting temperature of the polymer. It is most preferable to gradually increase the temperature of heat treatment in accordance with the increase of the melting temperature of the polymer during heat treatment.

The duration of the heat treatment will commonly range from a few minutes to a number of days, e.g., from 0.5 to 200 hours, or more. Preferably, the heat treatment is conducted for a time of 1 to 48 hours and typically from about 5 to 30 hours.

Generally, the duration of heat treatment varies depending upon the heat treatment temperature; that is, a shorter treatment time is required as a higher treatment temperature is used. Thus, the duration of the heat treatment can be shortened for higher melting polymers, since higher heat treatment temperatures can be applied without melting the polymer.

Preferably, the heat treatment is conducted under conditions sufficient to increase the melting temperature of the polymer at least 10 centigrade degrees. Most preferably, the melting temperature of the liquid crystal polymer is increased from between about 20 to about 50 centigrade degrees as a result of the heat treatment. The amount of increase which is obtained is dependent upon the temperature used in the heat treatment, with higher heat treatment temperatures giving greater increases.

It should be noted at this time that reference herein to a temperature below which a specific polymer may exhibit anisotropic properties in the melt phase is intended to refer to the temperature below which the polymer exhibits such properties prior to any heat treatment thereof.

The chemical resistance of the polymer also increases with heat treatment and the solubility into pentafluorophenol, one of the rare solvents for thermotropic liquid crystal polymers, continuously decreases with increasing heat treatment time and eventually the material will not dissolve even minimally (such as in amounts of 0.1 percent by weight).

The invention is additionally illustrated in connection with the following Examples which are to be considered as illustrative of the present invention. It should be understood, however, that the invention is not limited to the specific details of the Examples.

#### EXAMPLE 1

Several linear yards of a plain weave fabric containing 12½ ends per inch of 3000 filament carbon fiber yarn marketed by Union Carbide under the tradename Thornel T-300 in the warp direction and 12½ ends per inch of 3000 denier liquid crystal polymer yarn in the weft direction are woven. The liquid crystal polymer is comprised of 27 mole percent of a 6-oxy-2-naphthoyl moiety and 73 mole percent of a p-oxy benzoyl moiety. The

resulting fabric comprises approximately 33 volume percent carbon fiber and 67 volume percent of the liquid crystal polymer in filament form at approximately 6 denier per filament.

Four sections of the above fabric of 3×10 inches in dimension with the carbon fiber in the long direction are cut and stacked. The stacked sections of fabric are placed in a metal die mold of similar dimensions which is then placed in a heated press at 288° C. The press platens are brought into contact with the outer faces of the mold to enhance heat transfer to the mold. The mold is transferred to a water cooled press at ambient temperature after 45 minutes at 288° C. A pressure of 100 psi is applied to the stacked fabric in the mold and maintained for 30 minutes while the mold temperature is reduced to near ambient by the passage of cooling water through the press platens.

The laminated fabric thus formed is removed from the mold and determined to have a thickness of 0.026 inch. The laminate is relatively well compacted and exhibits no evidence of individual filaments of the liquid crystalline polymer. The filaments are completely fused and reformed to form a matrix for the carbon fiber yarn which exhibits minimal porosity. Tensile bars 8½ inches long in the carbon fiber direction and ½ inch wide are cut from the laminate. Tabs composed of fiberglass-reinforced epoxy 2½ inch×½ inch in dimension are attached to the ends of both faces by use of a commercial cyanoacrylate adhesive to protect the ends of the tensile bars from being crushed in the transverse direction during testing. These specimens are tested in an Instron test machine whereby they are determined to exhibit the following tensile properties by use of ASTM test method 1D3039:

|    | Tensile Strength<br>(psi) | Tensile Modulus<br>(psi) | Failure Elongation<br>(%) |
|----|---------------------------|--------------------------|---------------------------|
| 40 | 111,000                   | 10.4 × 10 <sup>6</sup>   | 1.1                       |

#### EXAMPLE 2

Fifteen sections or plies of a fabric produced in accordance with Example 1 are placed in a mold of dimensions 3×10 inches with the carbon fibers oriented in the long direction. A laminate is prepared by maintaining the mold at 288° C. with contact pressure for 2 hours. The laminate is held in a water-cooled press for 1 hour at 200 psi, whereby a laminate of 0.095 inch thickness is prepared containing 34 volume percent of carbon fiber. The short beam shear strength is measured using ASTM test method D2344 with a 4:1 span-to-depth ratio and determined to be 6500 psi.

#### EXAMPLE 3

Twelve sections or plies of a fabric prepared as in Example 1 are stacked in a 3×10 inch mold with the carbon fiber oriented in the long direction. A laminate is prepared by placing the mold and the charge in a heated press at 177° C. for 30 minutes under a pressure of 50 psi. The laminate is transferred to a water-cooled press and held under a pressure of 300 psi for 15 minutes. The laminate is removed and determined to have a thickness of 0.078 inches and a carbon fiber content of 34 volume percent. Flexural specimens of 4 inch lengths and ¼ inch widths are cut from the laminate. The mechanical properties of the specimens are measured by ASTM Test

Method D790 at a 32:1 span-to-depth ratio and the properties determined as follows:

| Flexural Strength<br>(psi) | Flexural Modulus<br>(psi) |
|----------------------------|---------------------------|
| 99,500                     | $8.8 \times 10^6$         |

The principles, preferred embodiments and modes of operation of the present invention have been described in the foregoing specification. The invention which is intended to be protected herein, however, is not to be construed as limited to the particular forms disclosed, since these are to be regarded as illustrative rather than restrictive. Variations and changes may be made by those skilled in the art without departing from the spirit of the invention.

We claim:

1. A fabric which exhibits thermal stability and chemical and solvent resistance comprised of fusible and infusible fibers, said fusible fibers being thermally bonded to said infusible fibers and comprised of a polymer which is capable of forming an anisotropic melt phase.

2. The fabric of claim 1 wherein said polymer is a wholly aromatic polymer.

3. The fabric of claim 1 wherein said polymer is a wholly aromatic polyester.

4. The fabric of claim 1 wherein said polymer exhibits an inherent viscosity of at least 2.0 dl./g. when dissolved in a concentration of 0.1 percent by weight in pentafluorophenol at 60° C.

5. The fabric of claim 1 wherein said polymer comprises not less than about 10 mole percent of recurring units which include a naphthalene moiety.

6. The fabric of claim 5 wherein said naphthalene moiety of said wholly aromatic polymer is selected from the group consisting of a 6-oxy-2-naphthoyl moiety, a 2,6-dioxynaphthalene moiety, and a 2,6-dicarboxynaphthalene moiety.

7. The fabric of claim 1 wherein said polymer is capable of forming an anisotropic melt phase at a temperature below approximately 400° C.

8. The fabric of claim 1 wherein said polymer comprises a melt processable wholly aromatic polyester which is capable of forming an anisotropic melt phase and consists essentially of the recurring moieties I, II, and III wherein:



wherein said polyester comprises approximately 30 to 70 mole percent of moiety I and wherein at least some of the hydrogen atoms present upon the rings optionally may be replaced by substitution selected from the group consisting of an alkyl group of 1 to 4 carbon atoms, an alkoxy group of 1 to 4 carbon atoms, halogen, phenyl, substituted phenyl, and mixtures thereof.

9. The fabric of claim 8 wherein said polyester comprises approximately 40 to 60 mole percent of moiety I, approximately 20 to 30 mole percent of moiety II, and approximately 20 to 30 mole percent of moiety III.

10. The fabric of claim 1 wherein said polymer comprises a melt processable wholly aromatic polyester which is capable of forming an anisotropic melt phase and consists essentially of the recurring moieties I and II wherein:



30 wherein said polyester comprises approximately 10 to 90 mole percent of moiety I, and approximately 10 to 90 mole percent of moiety II and wherein at least some of the hydrogen atoms present upon the rings optionally may be replaced by substitution selected from the group consisting of an alkyl group of 1 to 4 carbon atoms, an alkoxy group of 1 to 4 carbon atoms, halogen, phenyl, substituted phenyl, and mixtures thereof.

35 40 45 50 55 60 65 70 75 80 85 90 95 100 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685

percent of moiety II, and approximately 5 to 45 mole percent of moiety III and wherein at least some of the hydrogen atoms present upon the rings optionally may be replaced by substitution selected from the group consisting of an alkyl group of 1 to 4 carbon atoms, an alkoxy group of 1 to 4 carbon atoms, halogen, phenyl, substituted phenyl, and mixtures thereof.

14. The fabric of claim 13 wherein said polyester comprises approximately 20 to 80 mole percent of moiety I, approximately 10 to 40 mole percent of moiety II, and approximately 10 to 40 mole percent of moiety III.

15. The fabric of claim 1 wherein said polymer comprises a melt processable wholly aromatic polyester which is capable of forming an anisotropic melt phase and consists essentially of the recurring moieties I, II, III and IV wherein:



III is a dioxy aryl moiety of the formula  $-\text{O}-\text{Ar}-\text{O}-$  wherein Ar is a divalent radical comprising at least one aromatic ring, and



wherein Ar' is a divalent radical comprising at least one aromatic ring, and

wherein the polyester comprises approximately 20 to 40 mole percent of moiety I, in excess of 10 up to about 50 mole percent of moiety II, in excess of 5 up to about 30 mole percent of moiety III, and in excess of 5 up to about 30 mole percent of moiety IV and wherein at least some of the hydrogen atoms present upon the rings optionally may be replaced by substitution selected from the group consisting of an alkyl group of 1 to 4 carbon atoms, an alkoxy group of 1 to 4 carbon atoms, halogen, phenyl, substituted phenyl, and mixtures thereof.

16. The fabric of claim 15 wherein said polyester comprises approximately 20 to 30 mole percent of moiety I, approximately 25 to 40 mole percent of moiety II, approximately 15 to 25 mole percent of moiety III and approximately 15 to 25 mole percent of moiety IV.

17. The fabric of claim 1 wherein said polymer comprises a melt processable poly(ester-amide) which is capable of forming an anisotropic melt phase and consists essentially of the recurring moieties I, II, III and optionally IV wherein:



5 II is  $-\text{C}(=\text{O})-\text{A}-\text{C}(=\text{O})-$ , where A is a divalent radical comprising at least one aromatic ring or a divalent trans-cyclohexane radical;

III is  $-\text{Y}-\text{Ar}-\text{Z}-$ , where Ar is a divalent radical comprising at least one aromatic ring, Y is O, NH or NR, and Z is NH or NR, where R is an alkyl group of 1 to 6 carbon atoms or an aryl group; and

10 IV is  $-\text{O}-\text{Ar}'-\text{O}-$ , where Ar' is a divalent radical comprising at least one aromatic ring;

and wherein said poly(ester-amide) comprises approximately 10 to 90 mole percent of moiety I, approximately 5 to 45 mole percent of moiety II, approximately 5 to 45 mole percent of moiety III, and approximately 0 to 40 mole percent of moiety IV and wherein at least some of the hydrogen atoms present upon the rings optionally may be replaced by substitution selected from the group consisting of an alkyl group of 1 to 4 carbon atoms, an alkoxy group of 1 to 4 carbon atoms, halogen, phenyl, substituted phenyl, and mixtures thereof.

18. The fabric of claim 1 wherein said polymer has been subjected to a heat treatment for a period of time and at a temperature sufficient to increase the melting temperature of the polymer between about 20 to 50 centigrade degrees.

19. The fabric of claim 18 wherein said polymer has been subjected to a heat treatment after formation of said fabric.

20. The fabric of claim 18 wherein said heat treatment temperature ranges from about 10 to about 30 centigrade degrees below the melting temperature of the polymer.

21. The fabric of claim 20 wherein said period of time ranges from about 0.5 to about 200 hours.

22. The fabric of claim 21 wherein said period of time ranges from about 1 to about 48 hours.

23. The fabric of claim 22 wherein said period of time ranges from about 5 to about 30 hours.

24. The fabric of claim 18 wherein said heat treatment occurs in a non-oxidizing atmosphere.

25. The fabric of claim 24 wherein said atmosphere is substantially moisture-free.

26. The fabric of claim 24 wherein said heat treatment occurs in a nitrogen atmosphere.

27. The fabric of claim 1 which is in the form of a sheet.

28. The fabric of claim 1 wherein said infusible fibers are in the form of a woven web of said fibers.

29. The fabric of claim 1 wherein said infusible and fusible fibers are woven together to form said fabric.

30. The fabric of claim 1 wherein said fabric is formed by spray spinning said fusible fibers onto a web of infusible fibers and thermally bonding said fusible fibers to said infusible fibers.

31. The fabric of claim 1 wherein said fabric is formed by filtering a slurry of fusible and infusible fibers onto a web or screen and thermally bonding said fusible fibers to said infusible fibers.

32. The fabric of claim 1 wherein said infusible fibers are selected from the group consisting of carbon fibers, glass fibers and asbestos fibers.

33. The fabric of claim 32 wherein said infusible fibers are carbon fibers.

34. The fabric of claim 1 comprised of from about 5 to about 80 weight percent of infusible fibers and between about 95 to about 20 weight percent of fusible fibers.

\* \* \* \* \*